

## [54] HIGH STRENGTH TITANIUM ALLOYS

[75] Inventors: Warren Parris, Las Vegas; Harry W. Rosenberg, Boulder City, both of Nev.

[73] Assignee: Titanium Metals Corporation of America, West Caldwell, N.J.

[22] Filed: Apr. 18, 1972

[21] Appl. No.: 245,177

[52] U.S. Cl. .... 75/175.5

[51] Int. Cl. .... C22c 15/00

[58] Field of Search .... 75/175.5; 148/32, 133, 148/12.7, 11.5 F

## [56] References Cited

## UNITED STATES PATENTS

|           |         |                 |      |            |
|-----------|---------|-----------------|------|------------|
| 3,615,378 | 10/1971 | Bomberger       | .... | 75/175.5   |
| 2,804,409 | 8/1957  | Kessler et al.  | .... | 75/175.5 X |
| 2,819,959 | 1/1958  | Abkowitz et al. | .... | 75/175.5   |
| 2,884,323 | 4/1959  | Abkowitz et al. | .... | 75/175.5   |
| 2,892,706 | 6/1959  | Jaffee et al.   | .... | 75/175.5   |

3,436,277 4/1969 Bomberger et al. .... 148/12.7  
3,649,259 3/1972 Heitman .... 75/175.5

## OTHER PUBLICATIONS

Nuclear Science Abstracts, Vol. 22 No. 3, Feb. 15, 1968, Abst. No. 4762 & 4763.

Primary Examiner—Charles N. Lovell  
Attorney, Agent, or Firm—Webb, Burden, Robinson & Webb

## [57] ABSTRACT

A titanium base alloy comprising 6.3 – 11.0 percent vanadium, 1.75 – 3.3 percent aluminum, 0.75 – 2.25 percent iron, up to 2.25 percent chromium, up to 1.25 percent cobalt, up to 2.25 percent tin, up to 2.25 percent zirconium, up to 0.2 percent oxygen, balance titanium; the total of aluminum plus one half zirconium being between 2.25 percent and 3.25 percent, the ratio of iron to aluminum being no greater than about 1:1 and the maximum of iron plus cobalt being 2.25 percent.

3 Claims, No Drawings

## HIGH STRENGTH TITANIUM ALLOYS

This invention relates to high strength titanium base alloys and more particularly to titanium base alloys including vanadium, aluminum and iron as essential constituents with other elements included optionally. Various elements are included in the alloy in specified relationships which are set forth hereinafter.

Articles made from alloys within the composition range of our invention are deep hardenable and have high room temperature strength, good ductility, good notch strength and fracture toughness. The articles are age hardenable and heat treatable to high strength in thick sections. Additionally, the parts have good resistance to plane strain fracture.

In modern technology it is important to combine high strength with good ductility and good fracture toughness. For example, a metal which is not resistant to plane strain fracture may fail under stress due to the presence of a finite crack which is so small that it cannot be seen even in the presence of a dye penetrant. In order to obtain a high strength article, the alloy must

The base composition of our novel alloy consists essentially of 6.3 - 11% V, 1.75 - 3.3% Al, 0.75 - 2.25% Fe, balance titanium with a maximum oxygen content of 0.2 percent. The total amount of oxygen plus other incidental impurities should not exceed 0.35 percent. The iron to aluminum ratio in the alloy should not exceed about 1:1. Our alloy may optionally include up to 2.25 percent chromium, up to 1.25 percent cobalt, up to 2.25 percent tin and up to 2.25 percent zirconium. When zirconium is present in the alloy, the total of aluminum plus one half the zirconium will be between 2.25 percent and 3.25 percent. When cobalt is present in the alloy, the percent of cobalt plus the percent of iron should not exceed 2.25 percent since the cobalt replaces an equivalent amount of iron in the composition. Additionally, when chromium is included in the alloy, it should generally replace an equal amount of vanadium.

Table I shows a number of nominal titanium base alloy compositions, both within and outside the range of our invention, together with heat treatments and the results of metallurgical tests performed on these alloys.

TABLE I

TENSILE AND PLANE STRAIN TOUGHNESS PROPERTIES, TENSILE PROPERTIES  
TRANSVERSE,  $K_{IC}$  DATA FOR CRACK PROPAGATING IN DIRECTION OF ROLLING

| Heat                | Composition |     |     |             | Heat Treatment <sup>(1)</sup> | UTS | YS  | Lo El <sup>(2)</sup> | El <sup>(3)</sup> | $K_{IC}$                 |
|---------------------|-------------|-----|-----|-------------|-------------------------------|-----|-----|----------------------|-------------------|--------------------------|
|                     | V           | Fe  | Al  | Other       |                               | Ksi | Ksi | %                    | %                 | Ksi/ $\sqrt{\text{in.}}$ |
| 4505 <sup>(2)</sup> | 10          | 2   | 3   |             | As Rolled+1000F-4Hr-AC        | 186 | 181 | 20                   | 9                 | 51.6                     |
| do.                 | do.         | do. | do. |             | 1425F-1/4Hr-AC+1000F-4Hr-AC   | 194 | 187 | 15                   | 3                 | 49.7                     |
| 4543                | 10          | 2   | 3   |             | As Rolled+950F-4Hr-AC         | 181 | 170 | 30                   | 10                | 50.1                     |
| do.                 | do.         | do. | do. |             | 1400F-1/2Hr-AC+950F-8Hr-AC    | 179 | 171 | 20                   | 8                 | 52.3                     |
| do.                 | do.         | do. | do. |             | 1400F-1/2Hr-AC+1000F-2Hr-AC   | 178 | 170 | 25                   | 9                 | 55.3                     |
| 4550                | 10          | 3   | 2   |             | As Rolled+950F-8Hr-AC         | 180 | 176 | 30                   | 10                | 32.6                     |
| do.                 | do.         | do. | do. |             | 1400F-1/2Hr-AC+1000F-1Hr-AC   | 198 | 194 | 10                   | 4                 | 31.3                     |
| 4551                | 10          | 2   | 2   |             | 1400F-1/2Hr-AC+1000F-1Hr-AC   | 184 | 175 | 10                   | 2                 | 45.3                     |
| 4552                | 10          | 3   | 3   |             | 1400F-1/2Hr-AC+1100F-1Hr-AC   | 164 | 159 | 25                   | 14                | 67.6                     |
| 4554                | 10          | 2   | 3   | 1Zr         | As Rolled+950F-8Hr-AC         | 191 | 185 | 30                   | 12                | 37.2                     |
| do.                 | do.         | do. | do. |             | 1400F-1/2Hr-AC+1050F-1Hr-AC   | 180 | 172 | 20                   | 8                 | 44.2                     |
| 4555                | 10          | 2   | 3   | .1Zr        | 1400F-1/2Hr-AC+950F-4Hr-AC    | 194 | 184 | 20                   | 7                 | 43.0                     |
| 4556                | 10          | 1   | 3   | 1Co         | 1400F-1/2Hr-AC+900F-8Hr-AC    | 198 | 190 | 20                   | 6                 | 38.8                     |
| 4557                | 10          | 1   | 3   | 1Co-.1Zr    | 1400F-1/2Hr-AC+900F-8Hr-AC    | 200 | 191 | 20                   | 8                 | 40.1                     |
| 4506 <sup>(2)</sup> | 7           | 2   | 2   | 2Cr-2Sn-2Zr | As Rolled+1100F-2Hr-AC        | 187 | 186 | 10                   | 6                 | 57.6                     |
| do.                 | do.         | do. | do. |             | 1375F-1/2Hr-AC+1050F-2Hr-AC   | 187 | 179 | 10                   | 7                 | 58.4                     |

(1) As rolled from 1400F.

(2) 0.275" Plate finish rolled at 1450F, all others, 0.325" plate finish rolled at 1400F.

have sufficient fracture toughness to prevent failure in the presence of microscopic flaws. The alloys of our invention have this capability.

It is known in the art that the addition of beta stabilizers to a titanium base alloy results in good response to heat treatment and imparts high strength to the alloy. Additionally, it is known that the heat treatability and depth of hardening of an alloy increase in proportion to the amount of retained beta phase after quenching the alloy to room temperature. While the alloys of our invention follow these basic principles, it should be understood that we have discovered novel alloying combinations as discussed hereinafter. We have further discovered that direct aging of hot worked articles made from the novel alloys of our invention provides high ductility at ultimate strength to density ratios exceeding 1,100,000 inches. Our alloys have good fracture toughness even after solution treating in the alpha-beta field followed by aging.

50 A comparison of the data in Table I shows that Heat 4506 has the highest combination of yield strength and fracture toughness as indicated by  $K_{IC}$ . The alloy of Heat 4506 is based upon a substitution of 2%Cr for 3%V and 2%Sn +2%Zr for 1%Al. These substitutions strengthen both the alpha and beta phases in the alloy without substantially changing the ratio of the phases. This permits higher aging temperatures for a given desired strength level. The substitutions are also beneficial to fracture toughness.

60 As stated earlier, good fracture toughness is achieved by maintaining the iron to aluminum ratio below about 1:1 and by maintaining the aluminum plus one half the zirconium in the range of 2.25 percent to 3.25 percent. This can be seen by comparing the results of Heat 4550, wherein the iron to aluminum ratio is 3:2, and the results of Heats 4505 and 4543, wherein the iron to aluminum ratio is 2:3. Results of Heats 4555 and 4554 illustrate the effects of aluminum plus one half zirconium. These composition limitations may be seen

more clearly in Table II. In Table II the linear least squares analysis trend line values for  $K_{IC}$  for various heats were calculated and are compared with observed  $K_{IC}$  values. This data shows that an increase of the iron to aluminum ratio above 1:1 reduces the  $K_{IC}$  below expected values by at least 5 ksi  $\sqrt{\text{in.}}$  as does allowing the total of aluminum plus one half the zirconium to be outside the range of 2.25 percent to 3.25 percent.

It will also be seen from Table II that substitution of one cobalt for 1 percent iron as well as the addition of 0.1 percent zirconium results in an alloy having observed results close to the trend line.

TABLE II

| PLANE STRAIN TOUGHNESS VALUES<br>OBSERVED AND TREND LINE |    |    |             |                                   |                           |
|----------------------------------------------------------|----|----|-------------|-----------------------------------|---------------------------|
| Composition                                              |    |    |             | $K_{IC}$ -KSI $\sqrt{\text{in.}}$ |                           |
| V                                                        | Fe | Al | Other       | Observed                          | Trend Line <sup>(1)</sup> |
| 10                                                       | 2  | 3  |             | 49.7<br>52.3<br>55.3              | 41.9<br>54.2<br>54.9      |
| 10                                                       | 2  | 2  |             | 45.3                              | 51.1                      |
| 10                                                       | 3  | 2  |             | 31.3                              | 36.5                      |
| 10                                                       | 3  | 3  |             | 67.6                              | 63.4                      |
| 10                                                       | 2  | 3  | 1Zr         | 44.2                              | 53.4                      |
| 10                                                       | 2  | 3  | .1Zr        | 43.0                              | 44.2                      |
| 10                                                       | 1  | 3  | 1Co         | 38.8                              | 39.6                      |
| 10                                                       | 1  | 3  | 1Co-.1Zr    | 40.1                              | 38.8                      |
| 7                                                        | 2  | 2  | 2Cr-2Sn-2Zr | 58.4                              | 48.0                      |

(1) Calculated from linear least squares of solution treat plus age data given in Table I:  $K_{IC} = 185.42 - 0.7676 \text{ YS}$

As stated, the best  $K_{IC}$  performance is obtained by substituting 2 percent chromium for 3 percent vanadium and 2 percent tin plus 2 percent zirconium for 1 percent aluminum in the basic Ti-10V-2Fe-3Al alloy. The preferred compositions of our novel alloy are the

basic Ti-10V-2Fe-3Al alloy and Ti-7V-2Cr-2Fe-2Al-2Sn-2Zr. In both of these alloys, the preferred maximum oxygen content is 0.11 percent although oxygen may be present up to 0.2 percent. The total of oxygen and the other interstitials, carbon and nitrogen, may be present up to 0.35 percent.

In many applications the ability of a metal product to retain high strength in the presence of a machined notch is important. Table III shows the results of tests on  $\frac{1}{2}$  inch round bars finish rolled from 1,400°F and then subjected to high stress in the presence of machined notches. The alloys of our invention which exhibit good toughness as shown by the  $K_{IC}$  values also have high notch strength. The notch tensile strength of

the preferred Ti-7V-2Cr-2Fe-2Al-2Sn-2Zr is higher than the yield strength even when the yield strength is in excess of 200 ksi. Additionally, Table III shows the effect of thermomechanical processing history on the properties of alloys within the scope of our invention.

The effect is particularly evident from a consideration of the reduction of area values. Values of about 50 percent are typical when the alloys are rolled from 1,400°F and then aged directly to a yield strength within the range of 160 - 180 ksi.

It is also shown in Table III that, when finished rolled from 1,400°F, the basic Ti-10V-2Fe-3Al alloy is flexible with regard to subsequent heat treatment. This is an important commercial feature of our alloy since microstructure control is not always possible throughout heavy sections in industrial practice. For this reason, if solutionizing should occur in one portion of a large section of our alloy before the rest of that section is finished forged, the properties will still be uniform after aging. Known high strength commercial titanium base alloys do not include this feature.

TABLE III

| TENSILE AND NOTCH TENSILE PROPERTIES OF $1/2''$ ROUND |             |     |     |       |                             |     |     |    |    |                    |
|-------------------------------------------------------|-------------|-----|-----|-------|-----------------------------|-----|-----|----|----|--------------------|
| Heat                                                  | Composition |     |     |       | Heat Treatment              | UTS | YS  | RA | EL | NTS <sup>(1)</sup> |
|                                                       | V           | Fe  | Al  | Other |                             |     |     |    |    |                    |
| 4550                                                  | 10          | 3   | 2   | —     | As Rolled+950F-4Hr-AC       | 185 | 181 | 56 | 11 | 237                |
| do.                                                   | do.         | do. | do. | —     | As Rolled+1000F-2Hr-AC      | 179 | 176 | 57 | 17 | 236                |
| do.                                                   | do.         | do. | do. | —     | As Rolled+1050F-1Hr-AC      | 162 | 160 | 56 | 17 | 234                |
| do.                                                   | do.         | do. | do. | —     | 1400F-1/2Hr-AC+950F-4Hr-AC  | 202 | 194 | 15 | 9  | —                  |
| do.                                                   | do.         | do. | do. | —     | 1400F-1/2Hr-AC+1000F-2Hr-AC | 186 | 177 | 29 | 6  | 229                |
| do.                                                   | do.         | do. | do. | —     | 1400F-1/2Hr-AC+1050F-1Hr-AC | 164 | 158 | 40 | 14 | 221                |
| 4551                                                  | 10          | 2   | 2   | —     | As Rolled+950F-4Hr-AC       | 154 | 153 | 60 | 19 | 238                |
| do.                                                   | do.         | do. | do. | —     | 1400F-1/2Hr-AC+950F-4Hr-AC  | 192 | 186 | 9  | 3  | 160                |
| 4552                                                  | 10          | 3   | 3   | —     | As Rolled+950F-8Hr-AC       | 179 | 179 | 41 | 15 | 255                |
| do.                                                   | do.         | do. | do. | —     | As Rolled+1000F-4Hr-AC      | 172 | 172 | 56 | 18 | 244                |
| do.                                                   | do.         | do. | do. | —     | As Rolled+1050F-2Hr-AC      | 174 | 172 | 52 | 14 | 243                |
| do.                                                   | do.         | do. | do. | —     | 1400F-1/2Hr-AC+950F-8Hr-AC  | 212 | 210 | 6  | 4  | 133                |
| do.                                                   | do.         | do. | do. | —     | 1400F-1/2Hr-AC+1000F-4Hr-AC | 210 | 205 | 8  | 2  | 150                |
| do.                                                   | do.         | do. | do. | —     | 1400F-1/2Hr-AC+1050F-2Hr-AC | 196 | 192 | 13 | 5  | 190                |
| 4553                                                  | 10          | 2   | 3   | —     | As Rolled+950F-8Hr-AC       | 179 | 176 | 55 | 16 | 242                |
| do.                                                   | do.         | do. | do. | —     | As Rolled+1000F-4Hr-AC      | 173 | 170 | 57 | 17 | 241                |
| do.                                                   | do.         | do. | do. | —     | As Rolled+1050F-2Hr-AC      | 166 | 164 | 55 | 18 | 248                |
| do.                                                   | do.         | do. | do. | —     | 1400F-1/2Hr-AC+950F-8Hr-AC  | 177 | 170 | 55 | 17 | 211                |
| do.                                                   | do.         | do. | do. | —     | 1400F-1/2Hr-AC+1000F-4Hr-AC | 183 | 173 | 40 | 15 | 228                |
| do.                                                   | do.         | do. | do. | —     | 1400F-1/2Hr-AC+1050F-2Hr-AC | 174 | 167 | 46 | 14 | 219                |
| 4554                                                  | 10          | 2   | 3   | 1Zr   | As Rolled+950F-4Hr-AC       | 185 | 182 | 51 | 19 | 234                |
| do.                                                   | do.         | do. | do. | —     | As Rolled+1000F-2Hr-AC      | 179 | 175 | 44 | 15 | 237                |
| do.                                                   | do.         | do. | do. | —     | As Rolled+1050F-1Hr-AC      | 171 | 168 | 45 | 16 | 226                |
| do.                                                   | do.         | do. | do. | —     | 1400F-1/2Hr-AC+950F-4Hr-AC  | 200 | 189 | 17 | 8  | 161                |
| do.                                                   | do.         | do. | do. | —     | 1400F-1/2Hr-AC+1000F-2Hr-AC | 191 | 183 | 17 | 7  | 186                |
| do.                                                   | do.         | do. | do. | —     | 1400F-1/2Hr-AC+1050F-1Hr-AC | 192 | 184 | 25 | 12 | 196                |
| 4555                                                  | 10          | 2   | 3   | .1Zr  | As Rolled+950F-4Hr-AC       | 177 | 174 | 58 | 19 | 242                |
| do.                                                   | do.         | do. | do. | —     | As Rolled+1000F-2Hr-AC      | 166 | 164 | 60 | 19 | 240                |
| do.                                                   | do.         | do. | do. | —     | As Rolled+1050F-1Hr-AC      | 162 | 161 | 60 | 21 | 233                |
| do.                                                   | do.         | do. | do. | —     | 1400F-1/2Hr-AC+950F-4Hr-AC  | 188 | 179 | 31 | 11 | 228                |
| do.                                                   | do.         | do. | do. | —     | 1400F-1/2Hr-AC+1000F-2Hr-AC | 176 | 169 | 52 | 16 | 214                |
| do.                                                   | do.         | do. | do. | —     | 1400F-1/2Hr-AC+1050F-1Hr-AC | 175 | 169 | 51 | 16 | 225                |
| 4556                                                  | 10          | 1   | 3   | 1Co   | As Rolled+950F-8Hr-AC       | 170 | 169 | 61 | 20 | 234                |
| do.                                                   | do.         | do. | do. | —     | As Rolled+1000F-4Hr-AC      | 163 | 163 | 65 | 22 | 236                |
| do.                                                   | do.         | do. | do. | —     | As Rolled+1050F-2Hr-AC      | 158 | 156 | 61 | 17 | 232                |

TABLE III -Continued

## TENSILE AND NOTCH TENSILE PROPERTIES OF 1/2" ROUND

| Heat                | Composition |     |     |             | Heat Treatment              | UTS | YS  | RA | EL | NTS <sup>(1)</sup> |
|---------------------|-------------|-----|-----|-------------|-----------------------------|-----|-----|----|----|--------------------|
|                     | V           | Fe  | Al  | Other       |                             |     |     |    |    |                    |
| do                  | do.         | do. | do. | do.         | 1400F-1/2Hr-AC+950F-8Hr-AC  | 176 | 171 | 56 | 17 | 230                |
| do                  | do.         | do. | do. | do.         | 1400F-1/2Hr-AC+1000F-4Hr-AC | 173 | 167 | 49 | 16 | 229                |
| do                  | do.         | do. | do. | do.         | 1400F-1/2Hr-AC+1050F-2Hr-AC | 170 | 164 | 58 | 21 | 234                |
| 4557                | 10          | 1   | 3   | 1Co-.1Zr    | As Rolled+950F-8Hr-AC       | 170 | 169 | 54 | 17 | 240                |
| do.                 | do.         | do. | do. | do.         | As Rolled+1000F-4Hr-AC      | 167 | 167 | 59 | 20 | 235                |
| do.                 | do.         | do. | do. | do.         | As Rolled+1050F-2Hr-AC      | 159 | 158 | 63 | 20 | 235                |
| do.                 | do.         | do. | do. | do.         | 1400F-1/2Hr-AC+950F-8Hr-AC  | 179 | 176 | 42 | 14 | 238                |
| do.                 | do.         | do. | do. | do.         | 1400F-1/2Hr-AC+1000F-4Hr-AC | 175 | 172 | 32 | 13 | 232                |
| do.                 | do.         | do. | do. | do.         | 1400F-1/2Hr-AC+1050F-2Hr-AC | 166 | 163 | 56 | 18 | 222                |
| 4515 <sup>(2)</sup> | 10          | 2   | 3   | —           | As Rolled+1000F-2Hr-AC      | 184 | 180 | 51 | 16 | 248                |
| do.                 | do.         | do. | do. | —           | As Rolled+1000F-4Hr-AC      | 177 | 174 | 54 | 16 | 248                |
| do.                 | do.         | do. | do. | —           | 1450F-1/4Hr-AC+1000F-2Hr-AC | 192 | 183 | 20 | 9  | 218                |
| do.                 | do.         | do. | do. | —           | 1450F-1/4Hr-AC+1000F-4Hr-AC | 188 | 183 | 25 | 10 | 214                |
| 4506 <sup>(2)</sup> | 7           | 2   | 2   | 2Cr-2Sn-2Zr | As Rolled+1000F-4Hr-AC      | 208 | 204 | 27 | 12 | 248                |
| do.                 | do.         | do. | do. | do.         | As Rolled+1000F-8Hr-AC      | 208 | 205 | 32 | 13 | 232                |
| do.                 | do.         | do. | do. | do.         | 1450F-1/4Hr-AC+1000F-4Hr-AC | 216 | 211 | 7  | 5  | 215                |
| do.                 | do.         | do. | do. | do.         | 1450F-1/4Hr-AC+1000F-8Hr-AC | 210 | 200 | 9  | 5  | 219                |

(1) Notch acuity factor  $K_I=8$ .

(2) Finish rolled above beta transus, all others finished rolled below beta transus.

The alloys of our invention may be made by the conventional industrial technique of compacting sponge blended with the basic or master alloy, melting and remelting the blend in a vacuum or in an inert gas atmosphere followed by forming operations such as forging, rolling, drawing, etc. into the desired semi-finished product. The semi-finished product is then heat treated as necessary to enable finishing and material application. It will be found that the alloys of our invention are useful in the manufacture of aerospace vehicles and in other environments which require a high strength to density ratio.

While we have shown and described preferred embodiments of our invention, it should be understood that our invention may otherwise be embodied within the scope of the appended claims.

We claim:

1. A titanium base alloy consisting essentially of 6.3 – 11.0 percent vanadium, 1.75 – 3.3 percent aluminum,

0.75 – 2.25 percent iron, up to 2.25 percent chromium, up to 1.25 percent cobalt, up to 2.25 percent tin, up to 2.25 percent zirconium, up to 0.2 percent oxygen, balance titanium, the ratio of iron to aluminum in said alloy being no greater than about 1:1 and the total of the iron and the cobalt being not greater than 2.25 percent, the foregoing quantities being in terms of weight percent.

2. An alloy according to claim 1 consisting of 10 percent vanadium, 2 percent iron and 3 percent aluminum.

3. An alloy according to claim 1 consisting of 7 percent vanadium, 2 percent iron, 2 percent aluminum and including 2 percent chromium, 2 percent tin and 2 percent zirconium, said alloy characterized by a  $K_{IC}$  fracture toughness of at least 35 ksi/  $\sqrt{\text{in}}$ .

40

\* \* \* \* \*

45

50

55

60

65

UNITED STATES PATENT OFFICE  
CERTIFICATE OF CORRECTION

Patent No. 3,802,877 Dated April 9, 1974

Inventor(s) Warren M. Parris and Harry W. Rosenberg

It is certified that error appears in the above-identified patent and that said Letters Patent are hereby corrected as shown below:

In Table I after Footnote (2) insert the following:

--(3) Elongation to fracture of 0.2 inch length  
that includes the Fracture. --.

--(4) Total elongation over 1 inch gage length. --.

Signed and sealed this 30th day of July 1974.

(SEAL)

Attest:

McCoy M. GIBSON, JR.  
Attesting Officer

C. MARSHALL DANN  
Commissioner of Patents